

## UNITED STATES PATENT OFFICE

2,087,226

COTTON CLOTH HAVING ORNAMENTAL  
EFFECTS THEREON AND METHODS OF  
PRODUCING THE SAME

Harold I. Huey, Lincoln, and George E. Farragut,  
Pawtucket, R. I., assignors, by mesne assignments,  
to Heberlein Patent Corporation, New York, N. Y., a corporation of New York

No Drawing. Application August 15, 1935,  
Serial No. 36,386

8 Claims. (Cl. 8—20)

The present invention relates to cotton cloth having ornamental effects thereon and to methods of producing such cloth.

It has for some time been the practice in the art to form ornamental designs on cotton fabrics by applying thereto in selected areas a parchmentizing agent thereby rendering these areas transparent.

It is an object of our invention to provide such a fabric, the ornamental appearance of which is enhanced by permanent cockles or crinkles formed in the unparchmentized areas. It is a further object of our invention to enhance the ornamental appearance of such fabrics by providing in the transparent areas very slightly darker or shadowy lines or portions. It is a still further object of our invention to provide a process whereby these ornamental effects may readily be obtained.

Cotton fabrics having predetermined areas parchmentized, as heretofore produced, have been finished with the unparchmentized portions in a smooth condition. We have found that if these unparchmentized portions are permanently crinkled while the parchmentized portions remain substantially smooth, the design tends to be emphasized and to stand out and the ornamental appearance of the fabric is greatly enhanced. We have also found that a permanent crinkle effect, desirable for this purpose, may readily be produced upon unparchmentized portions of cotton cloth, by applying thereto a caustic, such as caustic soda lye, at spaced intervals. The unparchmentized fabric portions so treated with the caustic will shrink if the cloth is not held under tension, and the intervals of untreated fabric between the portions subjected to the caustic treatment will, due to the shrinking of the treated portions, pucker or crinkle up, assuming the form of separated raised dots or cockles. Cotton fabric so treated will retain permanently its crinkled form when washed.

Caustic, when applied to the parchmentized cotton areas, has little or no tendency to shrink the threads thereof and so may be applied to such areas in spaced bands without producing noticeable crinkles thereon. However, the caustic imparts an added sheer or transparency to the parchmentized design areas to which it is applied. When the caustic is applied to these areas in spaced bands, the added sheerness produced in the bands creates pleasing shadowy effects in the design areas.

We may produce the novel effects of our invention in the following manner: A light weight

cotton fabric, bleached and mercerized, is parchmentized (made permanently transparent) with sulphuric acid or other cellulose solubilizing agents in separated predetermined areas by any suitable method. Such methods are now well known to the art and need no description by us. The fabric is then washed and dried and a caustic is applied thereto at predetermined spaced intervals. Preferably for this purpose we employ a print roll to apply the caustic in lines, 10 but other well known means may be employed.

The degree of concentration of the caustic employed and the relative areas of the treated and untreated portions may be varied according to the effect desired. We have found, however, that a prominent and enduring cockle effect may be obtained in the unparchmentized portions of the fabric and a noticeable shadowy effect produced in the parchmentized areas by applying caustic soda of a concentration about 110° Twaddell, thickened by any suitable starchy material, in bands or stripes about  $\frac{1}{8}$ " wide and spaced apart about  $\frac{1}{8}$ ".

As mentioned above the cloth to be so printed may be a mercerized cotton. The formation of a design thereon with sulphuric acid will produce transparent areas. Where the caustic soda is applied in bands or otherwise to the design so formed, it will cause shrinking of the unparchmentized mercerized fabric in the design where it touches it. The fabric as the result of this process will then include in its design transparentized areas and shrunk untransparentized areas and adjacent areas which will be neither transparentized nor shrunk but will consist simply of the original mercerized fabric.

After the caustic has been applied, the treated fabric is allowed to stand for a few minutes without tension and is then given a hot water wash without tension, dried in a slack drier and framed to the desired width on a tenter.

The fabric may be dyed at any convenient stage of the treatment.

In some cases the fabric may be mercerized after the parchmentizing treatment when more sheerness and less shadowy effect is desired.

The cockled effect produced in the unparchmentized portions of the cloth serves to emphasize the design and at the same time imparts to the fabric as a whole a lacy appearance, 50 greatly enhancing the ornamental appearance of the cloth. The shadowy effects in the parchmentized portions further contribute to the pleasing appearance of the fabric.

Due to the presence of areas which have been 55

treated with neither shrinking agent nor acid, fabrics processed according to our invention are softer and more workable than is the case with fabrics whose entire area is treated with one or the other of these reagents.

We claim:

- 5 1. A cotton fabric having parchmentized areas and unparchmentized areas, the unparchmentized areas having shrunken portions and other unshrunken portions puckered and standing out in relief, the parchmentized areas being smooth and having portions more sheer than other portions.
- 10 2. A cotton cloth having a pattern in relief and composed of relatively smooth parchmentized areas and of unparchmentized areas permanently crinkled, said unparchmentized areas including strips of shrunken material and alternate strips of unshrunken material.
- 15 3. A cotton cloth having a pattern of smooth parchmentized areas and raised crinkled unparchmentized areas within said pattern, said raised unparchmentized areas being in part shrunk and in part unshrunk.
- 20 4. A process for treating cotton fabric which comprises parchmentizing the fabric in a pattern and shrinking parts of the unparchmentized areas within the pattern by a shrinking agent while preserving other adjacent parts of the unparchmentized areas unacted upon by said shrinking agent, thereby producing a permanent crinkled effect in the said unparchmentized areas.
- 25 5. A process of treating cotton fabric which comprises parchmentizing the fabric in a pattern with sulphuric acid and shrinking parts of the unparchmentized areas within the pattern by a caustic soda of mercerizing strength, while preserving other adjacent parts of the unparch-

mentized areas unacted upon by said caustic soda, thereby producing a permanent crinkled effect in the said unparchmentized areas.

6. A process of treating cotton fabric to produce patterns in relief, which comprises parchmentizing portions to form parchmentized areas and unparchmentized areas and subjecting narrow separated strips of said fabric to a strong caustic without tension, while preserving other adjacent parts of the unparchmentized areas unacted upon by said caustic, thereby producing a permanent crinkling in said unparchmentized areas while leaving the parchmentized areas smooth.

7. The process of treating cotton fabric to produce patterns in relief, which comprises parchmentizing separated portions to form parchmentized areas and unparchmentized areas and subjecting separated portions of said unparchmentized areas to a strong caustic without tension to produce a permanent crinkling in said unparchmentized areas only, washing out the caustic and drying the fabric without tension.

8. The process of treating cotton fabric to produce patterns in relief, which comprises parchmentizing separated portions to form parchmentized areas and unparchmentized areas and treating said fabric with a strong caustic without tension in spaced narrow lines that cross both the parchmentized areas and the unparchmentized areas, while preserving other adjacent parts of the unparchmentized areas unacted upon by said caustic, thereby producing a permanent crinkling in said unparchmentized areas while leaving the parchmentized areas smooth.

HAROLD I. HUEY.  
GEORGE E. FARRAGUT.

#### Certificate of Correction

Patent No. 2,087,226.

July 13, 1937.

HAROLD I. HUEY ET AL.

It is hereby certified that error appears in the printed specification of the above numbered patent requiring correction as follows: Page 1, second column, line 20, for "110°" read 100°; and that the said Letters Patent should be read with this correction therein that the same may conform to the record of the case in the Patent Office.

Signed and sealed this 17th day of August, A. D. 1937.

[SEAL]

LESLIE FRAZER,  
Acting Commissioner of Patents.

treated with neither shrinking agent nor acid, fabrics processed according to our invention are softer and more workable than is the case with fabrics whose entire area is treated with one or the other of these reagents.

We claim:

- 5 1. A cotton fabric having parchmentized areas and unparchmentized areas, the unparchmentized areas having shrunken portions and other unshrunken portions puckered and standing out in relief, the parchmentized areas being smooth and having portions more sheer than other portions.
- 10 2. A cotton cloth having a pattern in relief and composed of relatively smooth parchmentized areas and of unparchmentized areas permanently crinkled, said unparchmentized areas including strips of shrunken material and alternate strips of unshrunken material.
- 15 3. A cotton cloth having a pattern of smooth parchmentized areas and raised crinkled unparchmentized areas within said pattern, said raised unparchmentized areas being in part shrunk and in part unshrunk.
- 20 4. A process for treating cotton fabric which comprises parchmentizing the fabric in a pattern and shrinking parts of the unparchmentized areas within the pattern by a shrinking agent while preserving other adjacent parts of the unparchmentized areas unacted upon by said shrinking agent, thereby producing a permanent crinkled effect in the said unparchmentized areas.
- 25 5. A process of treating cotton fabric which comprises parchmentizing the fabric in a pattern with sulphuric acid and shrinking parts of the unparchmentized areas within the pattern by a caustic soda of mercerizing strength, while preserving other adjacent parts of the unparch-

mentized areas unacted upon by said caustic soda, thereby producing a permanent crinkled effect in the said unparchmentized areas.

6. A process of treating cotton fabric to produce patterns in relief, which comprises parchmentizing portions to form parchmentized areas and unparchmentized areas and subjecting narrow separated strips of said fabric to a strong caustic without tension, while preserving other adjacent parts of the unparchmentized areas unacted upon by said caustic, thereby producing a permanent crinkling in said unparchmentized areas while leaving the parchmentized areas smooth.

7. The process of treating cotton fabric to produce patterns in relief, which comprises parchmentizing separated portions to form parchmentized areas and unparchmentized areas and subjecting separated portions of said unparchmentized areas to a strong caustic without tension to produce a permanent crinkling in said unparchmentized areas only, washing out the caustic and drying the fabric without tension.

8. The process of treating cotton fabric to produce patterns in relief, which comprises parchmentizing separated portions to form parchmentized areas and unparchmentized areas and treating said fabric with a strong caustic without tension in spaced narrow lines that cross both the parchmentized areas and the unparchmentized areas, while preserving other adjacent parts of the unparchmentized areas unacted upon by said caustic, thereby producing a permanent crinkling in said unparchmentized areas while leaving the parchmentized areas smooth.

HAROLD I. HUEY.  
GEORGE E. FARRAGUT.

#### Certificate of Correction

Patent No. 2,087,226.

July 13, 1937.

HAROLD I. HUEY ET AL.

It is hereby certified that error appears in the printed specification of the above numbered patent requiring correction as follows: Page 1, second column, line 20, for "110°" read 100°; and that the said Letters Patent should be read with this correction therein that the same may conform to the record of the case in the Patent Office.

Signed and sealed this 17th day of August, A. D. 1937.

[SEAL]

LESLIE FRAZER,  
Acting Commissioner of Patents.

**Certificate of Correction**

Patent No. 2,087,226.

July 13, 1937.

**HAROLD I. HUEY ET AL.**

It is hereby certified that error appears in the printed specification of the above numbered patent requiring correction as follows: Page 1, second column, line 20, for "110°" read 100°; and that the said Letters Patent should be read with this correction therein that the same may conform to the record of the case in the Patent Office.

Signed and sealed this 17th day of August, A. D. 1937.

[SEAL]

**LESLIE FRAZER,**  
*Acting Commissioner of Patents.*